

April 28, 1936.

T. L. DUNBAR

2,038,925

## METHOD AND APPARATUS FOR THE TREATMENT OF FIBROUS MATERIAL

Filed Nov. 20, 1934



INVENTOR:

Thomas L. Dunbar  
C. E. Hammatt Jr.  
ATTORNEY

## UNITED STATES PATENT OFFICE

2,038,925

## METHOD AND APPARATUS FOR THE TREATMENT OF FIBROUS MATERIAL

Thomas L. Dunbar, Watertown, N. Y., assignor to  
Chemipulp Process, Incorporated, Watertown,  
N. Y., a corporation of New York

Application November 20, 1934, Serial No. 753,893

25 Claims. (Cl. 92—7)

The present invention relates to an improved method and apparatus for the treatment of fibrous material. Objects of the invention are the provision of improvements in the treatment 5 of fibrous material and apparatus therefor, resulting in greater yield and improvement in the quality of the pulp produced, and economies in operation. These improvements are applicable to both acid and alkali pulping processes, as will 10 hereinafter appear.

In the digestion of fibrous material, for example wood chips, for the production therefrom of pulp suitable for use in the manufacture of paper, organic acids formed in the cook have 15 been found to attack the pulp at the end of the cook. It has been the practice to neutralize these acids to some extent by a base in the cooking liquor. However, the presence of too much base in the cooking liquor is uneconomical, due 20 to the reaction of this base with the active ingredients of the cooking liquor. In accordance with my present invention I remove a part of the acid-forming constituents from the fibrous material before it reaches the digester, with the 25 result that there is less acid formed in the cooking process.

It is further important in the digestion of fibrous material that the digestion liquor should penetrate to the center of the chips before reaction starts. Unless this is the case, reaction 30 of the liquor with the outer part of the chips will weaken the liquor, so that that part thereof which eventually penetrates to the center of the chip becomes so weak that this part of the chip 35 is not completely cooked and the fibres are only partially liberated. But when complete penetration is accomplished before reaction starts, the digestion of each individual chip becomes uniform throughout. In my process the chips are 40 rendered more porous by the removal of water-soluble constituents therefrom before the chips come in contact with the digestion liquor. There results a better and quicker penetration of the chip by the cooking liquor, resulting in saving 45 of time, greater yield of pulp and decidedly improved quality thereof.

Furthermore, the chips are in my process brought to a uniform moisture content before being treated with the digestion liquor. 50 In brief, my invention comprises a process and apparatus in which fibrous material, for example wood chips, is first treated with water or other suitable solvent liquid at an elevated temperature. After this treatment the fibrous material is conveyed in the novel manner herein-

after described in detail, to a digester, where it is brought to complete fibre liberation by treatment with acid or alkaline liquor. The water in which the fibrous material is pretreated is drained from the fibrous material during the 5 passage from the pretreatment tank to the digester, and some of this water may be re-used in the pretreatment of a subsequent batch of raw material. Further details of my process and apparatus will become apparent as the description 10 proceeds.

In the accompanying drawing:

Fig. 1 is a diagrammatic elevation of apparatus suitable for use in the practice of my invention, certain parts being omitted for greater 15 clearness of illustration, and

Fig. 2 illustrates a modification thereof.

Referring to the drawing, and particularly to Fig. 1, 1 is a pre-treatment tank which is filled with the fibrous material, for example wood 20 chips, from a storage bin or conveyor (not shown). The tank 1 is provided with nozzles 2 for the admission of steam thereto. The pipe 3, provided with valve 4, admits a supply of hot water to the tank 1. The tank 1 communicates 25 through the valve 5 with the worm conveyor 6 in its casing 7. The worm 6 may conveniently be driven by the motor 8. The pipe 9, with valved branches 10, serves to admit steam into the worm conveyor 6. 30

The conveyor 6 communicates with the pump 11, which in turn communicates with a vertical conduit or leg 12. Steam may be admitted to the leg 12 through the pipe 13 with its valve 14.

The top of the leg 12 communicates with the 35 conduit 15, which may be a continuation of the leg 12, and this conduit 15 contains a strainer section 16. Collecting means 17 are provided in conjunction with the strainer 16, to collect water drained from the chips through the strainer. 40 The strainer section 16 communicates through the valve 19 with the line 18, which in turn communicates through the valve 19a with the interior of the digester 20.

The collecting apparatus 17 communicates 45 with a leg or trap 21, which trap communicates with a tank 22. A valved drain 25 from the leg 21 may go to the sewer or to tank 22. The tank 22 communicates through the pipe 23 and valve 24, with the pre-treatment tank 1. 50

The leg 21 is provided with a vent 26 into the tank 22, to prevent the leg from becoming gas bound. The tank 22 is also supplied with a vent 27 to the atmosphere.

The collecting apparatus 17 is provided with a 55

gas vent 28, having therein a valve 29, which communicates with the line 30 and thus through the check valve 31 with the seal leg or trap 32.

The digester 20 is provided with liquor circulation apparatus comprising the strainer 72 connecting through the valve 33 with the pump 34 and circulation line 35 which enters the bottom of the digester through the valve 36.

37 is the digester relief line, having therein the valve 38. This line communicates through the eductor 39 with the drop leg 40, which latter communicates through the valve 41 with the interior of the accumulator or storage tank 42. The valved steam line 61 may lead to steam coils 15 (not shown) within the tank 42 or may admit steam directly to the contents of the tank 42.

From the bottom of the accumulator or tank 42 the valved line 43 leads to the pump 44, which pump may force liquor from the accumulator 42 20 through the line 45 and valve 46 into the line 18.

The leg 32 terminates in a distributor 50 within the liquor storage tank 51. Liquor from the storage tank 51 may be led through the valved line 52 to the pump 53 and forced by this pump 25 through the line 54, valve 55, check valve 56 and the line 57 to the eductor 39, whence it is carried by the drop leg 40 to the accumulator 42. The pump 53 may also supply liquor to the leg 32 through the valved line 58.

30 The leg 32 is provided with the gas vent 59 to the storage tank 51 and also with the valved drain 60 to the tank 51.

In the alternate arrangement shown in Fig. 2, a worm conveyor 70 with its casing 71 may be 35 provided in the line 18 to force the raw material into the digester 20.

Operation in accordance with my invention may, for example, be as follows:

The pretreatment tank 1 is filled with the substance to be cooked, for example wood chips, from a storage bin or conveyor. Suitable solvent liquid such as hot water is admitted to the chips in the tank 1 through the line 3 and valve 4, and liquid may also be admitted from the tank 22 through 40 the line 23 and valve 24. Most of the liquid supplied to the tank 1 is fresh hot water through the pipe 3; the water in the tank 22 contains solubles which in limited amounts are advantageous in the pretreatment but only a limited amount of 45 this liquid, depending on mill conditions, is returned to the tank 1.

Steam is admitted to the tank 1 through the nozzles 2 and the fibrous material and water therein are brought to approximately the boiling point, 100° C. The length of time of treatment of the fibrous material in the tank 1 depends upon the grade of pulp which it is desired to produce and upon the raw material which is being treated and the temperature of the water. 50 In general the treatment of the fibrous material in the tank 1 may last from 2 to 5 hours.

After the previous charge in the digester 20 has been cooked and discharged into the blow pit (not shown), the worm conveyor 6 is started, 65 the valve 5 is opened and the pump 11 is also started. At this time steam is admitted into the worm conveyor through the line 9 and branches 10 and also into the vertical leg 12 through the line 13. This steam further treats the chips as 70 they are moved toward the digester, and in addition the steam through the line 9 assists the worm in moving the chips to the pump 11.

The hot pretreated chips and water are forced by the pump 11 to the top of the leg 12, whence 75 they pass through the leg 15 to the strainer sec-

tion 16. The mixture of raw material and water passes over the screen 16 where the water is drained off, this removal of water being assisted by the fact that the strainer and collecting apparatus are under pressure. The water, with dissolved impurities, is forced by this pressure through the leg 21 into the tank 22. The leg 21 maintains a pressure on the system so that cooking liquor supplied through the line 45 will not lose its strength, this being particularly necessary when bisulphite acid liquor is used in the cook. The collecting apparatus 17 communicates through the vent 28, line 30, and valve 31 with the seal leg 32 which again is provided to maintain pressure on the system.

The pressure maintained by the seal legs 21 and 32 not only maintains the strength of the cooking liquor, but also assists the penetration of this liquor into the raw material being treated. This rapid penetration of the liquor into the material saves time, assists materially in delignification of the fibres and also increases the yield of the pulp. Whereas in the cold acid method of cooking considerable time should be taken to bring the mass in the digester up to a reaction 25 temperature of 110 to 120° C., in order to assure thorough penetration of the individual chips by the cooking liquor, in my preferred process this time is greatly reduced due to the rapidity of the penetration, which is assisted by the porous condition of the chips, their uniform moisture content, pressure and the elevated temperature of the liquor.

As previously stated, the chips may, if desired, be forced into the digester by a worm conveyor 30 35 as shown in Fig. 2.

While the pretreated material is entering the digester 20 through the line 18, cooking liquor from the accumulator or storage tank 42 is supplied thereto by the pump 44 and line 45. When 40 the digester 20 has been filled with chips and either hot or cold acid, the valve 19 is closed and additional cooking liquor is forced into the digester by the pump 44 until liquor flows free 45 through the relief valve 38 and the line 37 back to the accumulator, at which time the valve 38 is closed and a pressure is pumped on the digester by the pump 44. This pressure may be anywhere from 40 to 122 pounds gauge, depending upon 50 local plant conditions.

When the proper digester pressure has been attained, the pump 44 is stopped, the valve 19a is closed and steam is admitted at the bottom of the digester in the usual way through the conventional steam connections (not shown) which are 55 normally made to the blow off elbow. At the same time the valves 33 and 36 are opened and the pump 34 is started, which circulates the digester liquor through the strainer 72 and circulation line 35 into the bottom of the digester through the valve 36. This circulation may be continuous throughout the cooking period or may be intermittent. Its object is to provide more uniform 60 conditions of temperature and liquor concentration throughout the mass undergoing cooking in 65 the digester.

During the cook, the relief valve 38 and the customary side relief valve (not shown) are operated in the usual manner to withdraw the necessary liquors, gases and vapors from the digester 70 to the eductor 39 and accumulator 42. The eductor 39 is similar to that shown and described in Patent No. 1,888,632, issued November 22, 1932 to me and A. D. Merrill. This eductor is supplied with partially prepared acid from the storage tank 75

51 by the pump 53 and lines 54 and 57. The contacting of this relatively cold liquor with the relief fluids from the digester results in absorption of the relief fluids and reduces the back pressure on the relief line 37.

42 may be either a hot acid accumulator under super-atmospheric pressure or the ordinary storage tank under atmospheric pressure. In the latter case, the relief line 37 will be provided with 10 a cooler so that the liquor entering the tank 42 will be cooled and thus there will be less tendency for gases to escape therefrom. Or the tank 42 may be designed to withstand low pressures being for 15 example a reinforced concrete tank provided with an acid-proof lining in the case of the acid cooking process. If the tank is so designed to withstand low pressures, the cooler in the line 37 need not be of such large capacity as if the tank 42 is at atmospheric pressure.

20 In the case of the alkaline pulping process, the seal legs 21 and 32 may still be used to obtain pressure on the line 18 and thus to secure the advantage of proper penetration of the raw material by the cooking liquor. In the alkaline process, 25 the tank 42 may be provided with heating coils or steam may be admitted directly thereto to bring the temperature of the cooking liquor up to at least the temperature of the raw material entering the digester.

30 I prefer to have the temperature of the liquor entering the digester higher than that of the chips and I have found that the temperature of the liquor in the tank or accumulator 42 can be maintained as high as 130° C. without premature initiation of cooking of the chips, since the addition of cooking liquor at 130° C. to the raw material at 100° C. will result in a temperature of the mass at which thorough penetration is obtained before reaction temperatures are actually reached.

40 The legs or traps 21 and 32 are of a proper height to meet different pressure conditions due to variations in liquor concentration required by different mills. This is particularly so in the case of the acid cooking process since the concentration of the liquor is proportional to the temperature and pressure.

The vent 26 into the tank 22 prevents the seal leg 21 from becoming gas bound and this vent 26 conserves heat units contained in the hot gases 50 or air from the leg 21. Similarly, the vent 59 to the storage tank 51 prevents the leg 32 from becoming gas bound.

The leg 21 may be drained through the drain elbow 25 whenever necessary. The liquor so removed may be led to the sewer or may be pumped into the tank 22. The leg 32 is similarly provided with a drain 60. The distributor 50 at the bottom of the tank 51 ensures proper distribution of any liquor forced into this tank through the 60 leg 32.

65 My invention not only makes possible improved yield and quality of pulp but also results in economies in operation as compared with methods heretofore employed in the treatment of fibrous material.

Having thus described my invention, I claim:

1. In apparatus of the character described, a digester, a pretreatment tank, a conduit for fibrous material connecting the pretreatment tank 70 with the digester, a worm conveyor interposed in said conduit, and means for injecting steam into said pretreatment tank and into said conduit.

2. In apparatus of the character described, a digester, a pretreatment tank for fibrous material, 75 and a vertical conduit for fibrous material con-

necting with the pretreatment tank and with the digester, said conduit provided with a worm conveyor for forcing therethrough a fluent mixture of fibrous material and treating liquid from the pretreatment tank against the head of the material in said vertical conduit.

3. In apparatus of the character described, a digester, a pretreatment tank provided with means for supplying liquid thereto, a conduit for fibrous material connecting the pretreatment tank 10 with the digester, said conduit having interposed therein a worm conveyor, and means for injecting steam into said conduit between the pretreatment tank and the digester.

4. In apparatus of the character described, a 15 digester, a container for fibrous material, a worm conveyor connecting with the container for fibrous material, a pump connecting with the worm conveyor, and a conduit connecting said worm and said pump with the digester. 20

5. Apparatus as described in claim 4, including means for injecting steam into the worm conveyor and into the conduit.

6. In apparatus of the character described, a digester, a pretreatment tank, a conduit connecting the pretreatment tank with the digester and having interposed therein means for separating liquid from fibrous material, and a trap 25 for collecting liquid so separated and passing the same to the pretreatment tank while maintaining 30 fluid pressure on the separating means.

7. In apparatus of the character described, a digester, a pretreatment tank, a conduit connecting the pretreatment tank with the digester, said conduit provided with a strainer and with 25 means for collecting liquid separated by the strainer, and means for maintaining pressure within the conduit and collecting means while withdrawing liquid therefrom.

8. In apparatus of the character described, a 40 digester, a pretreatment tank, a conduit connecting the pretreatment tank with the digester, a trap communicating with said conduit and adapted to permit the escape of gas therefrom while maintaining pressure therein, and a second 45 trap communicating with said conduit and adapted to permit the escape of liquid therefrom.

9. In apparatus of the character described, a digester, a container for fibrous material, a conduit connecting the said container with the 50 digester, a strainer interposed in said conduit, collecting means for liquid separated by the strainer, said collecting means communicating through a trap with a storage tank for said liquid, and a gas vent from the trap to said storage 55 tank.

10. In apparatus of the character described, a digester, a pretreatment tank, a conduit for fibrous material connecting the pretreatment tank with the digester, a storage receptacle for digestion liquor, and means for passing digestion liquor from said storage receptacle into said conduit between the pretreatment tank and the digester. 60

11. In apparatus of the character described, a digester, a pretreatment tank, a conduit connecting the pretreatment tank with the digester, said conduit having interposed therein a strainer for separating liquid from fibrous material passing therethrough, a storage receptacle for digestion liquor, and means for passing digestion liquor 70 from said storage receptacle into said conduit between the strainer and the digester.

12. In apparatus of the character described, a digester, a pretreatment tank, a conduit connecting the pretreatment tank with the digester 75

and a trap communicating with said conduit and adapted to maintain pressure therein while permitting the escape of gas therefrom.

13. In apparatus of the character described, a digester, a pretreatment tank, a conduit connecting the pretreatment tank with the digester, a storage receptacle for liquor, a trap communicating with the conduit and terminating in a liquor distributor within said storage receptacle, 10 and a gas vent from said trap to said storage receptacle.

14. In apparatus of the character described, a digester, a pretreatment tank, a conduit connecting the pretreatment tank with the digester, 15 a trap communicating with said conduit, a storage receptacle for liquor, and means for supplying liquor from said storage receptacle to said trap.

15. The process of treating fibrous material 20 which comprises initially removing acid-forming constituents of the material and increasing the porosity thereof by immersing the material in water and injecting steam into the resulting mass, removing the fibrous material from the initial 25 treatment chamber and injecting additional steam thereinto while passing the material to a digester and thereafter digesting the material to complete fibre liberation in acid liquor.

16. The process of treating fibrous material 30 which comprises removing acid-forming constituents of the material by treatment of the material with heated water, straining water from the material while maintaining the same under fluid pressure and thereafter cooking the material 35 to complete fibre liberation in a single type of digestion liquor.

17. The treatment of fibrous material which 40 comprises removing water-soluble constituents therefrom by treating the material with heated water, then conveying the material so treated to a digester and injecting steam into the material during its passage from the water treatment to the digester, and thereafter cooking the material under heat and pressure to liberate the 45 fibres thereof.

18. The treatment of fibrous material which 50 comprises initially removing acid-forming constituents of the material and increasing the porosity thereof by treatment of the material in a heated solvent liquid, said treatment including forcing said material in the presence of the solvent liquid and of steam vertically through a conduit against the head of the mixture, and subsequently cooking the material to complete 55 fibre liberation in acid liquor under heat and pressure.

19. The process of treating fibrous material 60 which comprises increasing the porosity of the material and removing acid-forming constituents thereof by treating the same with water to liberate said constituents, treating the material with steam while conveying it to a strainer, and thereafter straining the material to remove water and liberated acid-forming constituents, and

finally cooking the material under heat and pressure to liberate fibres thereof.

20. The treatment of fibrous material which 5 comprises initially increasing the porosity of the material and removing acid-forming constituents therefrom by treating the material with water containing limited amounts of acid forming constituents extracted from a previous batch of similar material, and thereafter digesting the material to complete fibre liberation. 10

21. The process of treating fibrous material which 15 comprises removing acid-forming constituents therefrom by pretreatment of a first batch of such material with heated water, draining from the material said water with contained acid-forming constituents, cooking the pre-treated material to liberate the fibres thereof, and pretreating a subsequent batch of fibrous material with water and contained constituents drained from said first batch of material. 20

22. In the treatment of fibrous material, 25 pretreating such material in heated liquid to liberate acid-forming constituents therefrom, passing the pretreated material to a strainer and straining therefrom the pretreatment liquid containing acid-forming constituents, thereafter introducing 30 digestion liquor into the fibrous material, and maintaining the fibrous material under gaseous pressure during the said straining and during the introduction of said digestion liquor. 30

23. In a process for the treatment of fibrous material, subjecting fibrous material to pretreatment to liberate acid-forming constituents therefrom, adding digestion liquor to the pretreated fibrous material, and thereafter introducing the mingled fibrous material and digestion liquor into a digestion chamber. 35

24. In a process of the character described, subjecting fibrous material to pretreatment in 40 heated liquid to liberate acid-forming constituents of said material and to increase the porosity thereof, straining from the fibrous material pretreatment liquid with contained acid-forming constituents and returning said liquid to the pretreatment of a subsequent batch of fibrous material, adding heated digestion liquor to the fibrous material, then passing the fibrous material and digestion liquor to a digestion chamber and therein cooking the said material in the said liquor to liberate the fibres of the material. 45

25. In the treatment of fibrous material, subjecting fibrous material to pretreatment to liberate acid-forming constituents therefrom and increase the porosity thereof, said pretreatment involving heating the material to a temperature 55 in the neighborhood of 100° C., adding digestion liquor heated to a temperature above 110° C. to the porous pretreated fibrous material while said material is at a temperature in the neighborhood of 100° C., then raising the temperature of the 60 resulting mixture above 110° C. to initiate reaction of the liquor with constituents of the fibrous material.

THOMAS L. DUNBAR.